

Aug. 23, 1932.

P. R. YOUNG

1,873,098

SURFACE COVERING MATERIAL

Filed April 20, 1929

*Fig. 1.*



*Fig. 2.*



*Fig. 3.*



Paul R. Young  
by his attorney  
Byron, Stilman & Farrelly

## UNITED STATES PATENT OFFICE

PAUL R. YOUNG, OF LITITZ, PENNSYLVANIA, ASSIGNOR TO ARMSTRONG CORK COMPANY, OF LANCASTER, PENNSYLVANIA, A CORPORATION OF PENNSYLVANIA

## SURFACE COVERING MATERIAL

Application filed April 20, 1929. Serial No. 356,704.

This invention relates to surface covering material and is particularly adapted for use on the running boards of automobiles, although it has numerous other applications.

- 3 Auto mat material as used on the running boards of automobiles must withstand considerable wear—it must be water-proof, and must be resistant to sunlight and rain, as well as to wide extremes of temperature.
- 10 Linoleum compositions, particularly those having as a major ingredient pitch such as stearine pitch, has been found to be particularly desirable. Such material is more specifically described and claimed in the pending application of S. H. Hartman, Serial No. 304,613, filed Sept. 7, 1928. Such material is preferably calendered onto a water-proof paper backing, as described in Humphreys Patent No. 1,129,571.

20 A preferred composition is as follows:

|                                   | Parts      |
|-----------------------------------|------------|
| Linoleum cement                   | 90         |
| Stearine pitch                    | 120        |
| 25 Mineral filler such as whiting | 100        |
| Lime                              | 1          |
| Manganese resinate                | 1          |
| Ground cork                       | 100        |
| Linoleum scrap                    | 450 to 500 |

- 30 To the above may be added 12 parts of carbon-black to insure a black color. All of the above proportions are by weight. It is desirable to have a black composition as this permits of using linoleum scrap of any color. This composition, because of its high pitch content, is affected but little if any, by ultra-violet light. There is therefore no tendency toward disintegration from direct sunlight, as is the case in ordinary linoleum mixtures.
- 40 The above mix is also highly water-resistant and will withstand considerable scuffing and abrasion. It is very little affected by expansion and contraction and bonds readily with 45 the paper base.

Automobile manufacturers require a ribbed surface for their auto mat material, not only because of its improved appearance, but also because it gives a desirable tread surface.

- 50 In calendering mixtures suitable for auto

mat use, there is a tendency for the bottom of the grooves between ribs to roughen. The ribbed calender roll is set to slip on the face of the goods so as to give something of a burnishing action and thus secure a smooth 55 face, but while this result is obtained on the ribs themselves, the grooves therebetween show depressions somewhat resembling pock marks. This destroys the appearance of the entire product and because of the roughened 60 surface, it is likely to decrease the life of the material. Water lying on the running board of the car can get into the pits or depressions of the roughened groove bottoms and upon 65 freezing cause damage which, although slight, will, if repeated a sufficient number of times, ultimately affect the life and appearance of the mat.

I provide for placing a paint-like material in the corrugations so as to fill the pits 70 therein and provide a smooth surface. The paint-like material employed is preferably one which has a solvent action on the binder of the body material. When the filler material has such solvent action this fact, coupled with the roughness of the grooves, results 75 in the filler material being firmly keyed to the body. In fact, flexing of the material shows that the paint-like material very firmly adheres to the bottoms of the grooves. 80

The paint employed is preferably opaque so as to entirely hide the pits. Preferably it is not of sufficient thickness to entirely fill the grooves. The ribs therefore take all of the wear and the paint is not subjected to 85 scuffing. It will therefore preserve its surface appearance indefinitely. By using a paint of a contrasting color, very desirable effects may be obtained.

In the accompanying drawing illustrating 90 the present preferred embodiment of the invention as applied to auto mat material.

Figure 1 is a top plan view of a portion of the material with part of the paint-like 95 filler removed so as to show the pits at the bottoms of the grooves,

Figure 2 is a transverse section showing paint in some of the grooves, but with one groove unpainted, and 100

Figure 3 is a diagrammatic view illustrating the manner of applying the paint.

The material shown in the drawing comprises a base 2 of felt paper or the like, suitably water-proofed and having a body material 3 of a thermo-plastic mix such as above described, calendered thereon. The calender roll is shaped to provide ribs 4 alternating with grooves 5.

10 In Figure 1 I have illustrated at 6 the pits or depressions which are formed in the bottoms of the grooves by the calendering operation. In order to cover these pits, a paint-like material preferably employed is a nitro-cellulose lacquer. This has a solvent action 15 on the binder of the thermo-plastic material, and attaches itself very well thereto. Any desired paint may be used but it is preferably of a flexible character.

20 Figure 3 shows diagrammatically the manner of applying the paint to the grooves. The material is pulled under a flat edged rubber doctor blade 8 which lies at an angle to the direction of travel of the material.

25 A pool of lacquer L is placed in front of the doctor blade and as the material is pulled thereunder a lacquer film of the proper depth is laid in the grooves 5. Those portions of the edge of the doctor blade which lie over 30 the grooves in the material determine the depth of the lacquer therein. Those portions of the blade which lie over the ribs wipe the tops thereof clean so that the body material is exposed on the tops of the ribs to 35 form the wearing surface.

The paint contains a large percentage of volatile solvent, and when this evaporates, a film of desired thinness lays over the bottom and sides of the ribs. The irregularities of 40 the grooves are overcome and the exposed surface of the paint is smooth. The paint, after drying, does not fill the recesses but conforms generally to the shape thereof as indicated by dotted lines at the right-hand 45 side of Figure 2. The invention gives the desired ribbed effect with an additional decorative quality arising from the contrast afforded by the colored lacquer and the body material.

50 As above stated, the paint material employed preferably has a solvent action on the binder of the body material. One lacquer mix is here given by way of example only, as indicating a type of paint which will have 55 a solvent action on the material:

|                     | Parts |
|---------------------|-------|
| Nitrated cotton     | 10    |
| Ester gum           | 10    |
| Tricresyl phosphate | 1     |
| Castor oil          | 4     |
| Ethyl acetate       | 25    |
| Absolute alcohol    | 50    |

The above proportions are by weight. A suitable amount of pigment is added to the

above mix. Various other paints may, of course, be employed.

I have illustrated and described the present preferred embodiment of the invention. It will be understood, however, that it is not limited to the form shown but may be otherwise embodied within the scope of the following claims.

I claim:

1. An auto mat material comprising a body 75 of varying thickness having a face with recesses formed therein, and an opaque lacquer lying in the recesses.

2. An auto mat material comprising a body 80 having a generally plane back and a corrugated face, and a paint-like material lying in the corrugations but only partially filling the same.

3. A surface covering material comprising 85 a body of thermo-plastic material having a face with recesses formed therein, and a covering material lying in the recesses but only partially filling the same, the applied covering material having a solvent action on the body material.

4. A surface covering material comprising 90 a body of thermo-plastic material having recesses therein, the recesses having the characteristic irregularities resulting from calendering such material, and a paint filling such 95 irregularities.

5. A surface covering material comprising 100 a body of thermo-plastic material having recesses therein, the recesses having the characteristic irregularities resulting from calen- 100 dering such material, and a paint filling such irregularities and extending over the face of the recesses.

6. A surface covering material comprising 105 a body having ribs formed on a surface thereof, the spaces between the ribs having the characteristic irregularities resulting from the calendering of such material, and a paint filling such irregularities and extending over the surfaces between the ribs, the top faces of 110 the ribs being uncoated.

7. An auto mat material comprising a body having a generally plane back and a top surface with ribs formed thereon, the depressions between the ribs having pits or the like 115 therein, and a paint filling said pits and largely filling the depressions between the ribs.

8. An auto mat material comprising a body having a generally plane back and a top surface with parallel ribs extending continuously therealong so as to form a series of grooves between the ribs extending the length of the material, the grooves having pits or the like 120 therein, and a paint lying in the grooves and anchored in the pits, the paint largely filling 125 the grooves but the top surface of the paint lying below the top surface of the ribs.

9. An auto mat material comprising a body having a generally plane back and a corrugated face and a paint-like material lying in 130

the corrugations, the paint largely filling the corrugations but the surface of the paint lying below the level of those portions of the material between the corrugations.

5 In testimony whereof I have hereunto set my hand.

PAUL R. YOUNG.

10

25

20

25

30

35

40

45

50

55

60

65